

# UNITED STATES PATENT OFFICE.

THEODORE H. BROWN AND HAUGHTON BROWN, OF MINNEAPOLIS, MINNESOTA.

## COMPOSITION FOR ROOF AND WALL COVERING.

1,369,911.

Specification of Letters Patent.

Patented Mar. 1, 1921.

No Drawing.

Application filed April 19, 1920. Serial No. 374,868.

*To all whom it may concern:*

Be it known that we, THEODORE H. BROWN and HAUGHTON BROWN, citizens of the United States, residing at Minneapolis, in 5 the county of Hennepin and State of Minnesota, have invented certain new and useful Improvements in Compositions for Roof and Wall Covering; and we do hereby declare the following to be a full, clear, 10 and exact description of the invention, such as will enable others skilled in the art to which it appertains to make and use the same.

Our invention provides a new composition 15 which may be very cheaply made and which is highly efficient when used as a roof covering or as an inner or outer wall covering or for similar purposes.

This improved composition is made from 20 ashes (either coal or wood, mixed with fine cinders) asphalt (preferably gilsonite), vegetable fiber (waste broom straw) cut into short lengths.

The proportions of these materials may 25 be varied and will vary for different purposes, but I have made a material highly efficient for external roof and wall covering by using approximately fifty per cent. of ashes, twenty-five per cent. of asphalt 30 and twenty-five per cent. of vegetable fiber, the fiber being waste broom straws and the proportions stated, being in respect to bulk.

In making this composition, we first heat and melt the asphalt, then put ashes on top 35 of the molten asphalt and stir the same in while the asphalt is still at high temperature. Into the mixture thus produced, the cut or finely broken particles of the waste broom straw are thoroughly stirred in until 40 quite evenly distributed throughout the mass.

It is important that the broom straw be stirred in after the ashes have been thoroughly saturated by the hot asphalt and 45 the mass slightly cooled so that the broom straw will not be ignited or scorched or its fibers otherwise damaged.

When this commingled mass is thoroughly cooled, it will be quite hard but of such plastic nature that it may be given the desired 50 form by the pressure of forming rollers. This material, after it has been applied or otherwise formed, will harden somewhat by drying but will always have such elastic 55 character that it will adapt itself to shrinkage or expansion on plaster, concrete or lum-

ber, under varied conditions of moisture or temperature, and hence will not crack. The material is perfectly water proof, and almost fireproof and moreover is a good heat insulator. 60

The cut waste broom straws not only increase the tensile strength of the material, but further increase its heat insulating quality and makes the material lighter than it 65 would be if the straws were omitted.

This material will adhere well to plaster, concrete, wood, metal, or almost any other substance, if applied thereto while hot and on dry surface. 70

The lengths into which the broom straws will be cut will depend somewhat on the nature of the article that is being made or the manner in which the material is to be applied. When the material or composition 75 is to be applied with a trowel or is to be made, for example, in an imitation of shingles, the straws should be cut into short lengths, say from one-half to a quarter of an inch. But when the material is being 80 pressed into sheets by use of rollers for example, the straws may vary from short lengths to lengths as much as several inches, say six or eight inches.

To adapt the material to be more easily 85 spread on a surface, by use of a trowel, a little molasses may be advantageously added to the mixture above described.

It is important to note that all the main substances of the above material are of low 90 cost. The ashes and cinders and the waste broom straw, which constitute about three-fourths of the substance, are of little or no cost, and the asphalt is a very cheap material. The efficiency of this material, both 95 as inside and outside coverings, applied with the trowel and in the form of sheets and also in the form of shingles, have been thoroughly demonstrated in practice.

What we claim is: 100

1. A new compositional matter composed of ashes, fine cinders, asphalt and waste broom straw thoroughly commingled.

2. A new compositional matter comprising ashes, asphalt and vegetable fiber, the 105 ashes in bulk being about equal to the combined bulk of the asphalt and fiber.

3. A new compositional matter comprising ashes, asphalt and vegetable fiber, the ashes in bulk being about equal to the combined bulk of the asphalt and fiber and a 110 small amount of molasses.

4. A new compositional matter composed of approximately fifty per cent. of ashes and fine cinders, twenty-five per cent. of asphalt and approximately twenty-five per cent. of
5. finely cut waste broom straws or stalks thoroughly commingled.
5. A new compositional matter composed of approximately fifty per cent. of ashes and fine cinders, twenty-five per cent. of asphalt

and approximately twenty-five per cent. of 10 finely cut waste broom straws or stalks thoroughly commingled, and a small amount of molasses.

In testimony whereof we affix our signatures.

THEODORE H. BROWN.  
HAUGHTON BROWN.